

Jan. 21, 1964

F. R. CRAMTON

3,118,161

FOAMED POLYPROPYLENE FILAMENTS

Filed March 13, 1963

2 Sheets-Sheet 1



FIG. 1



FIG. 5 INVENTOR  
FRANK R. CRAMTON

BY *Beale & Jones*

ATTORNEY

Jan. 21, 1964

F. R. CRAMTON

3,118,161

FOAMED POLYPROPYLENE FILAMENTS

Filed March 13, 1963

2 Sheets-Sheet 2



INVENTOR

FRANK R. CRAMTON

BY *Beale & Jones*

ATTORNEY

**1**

3,118,161

FOAMED POLYPROPYLENE FILAMENTS  
Frank R. Cramton, Burlington, Vt., assignor to E. B. &  
A. C. Whiting Company  
Filed Mar. 13, 1963, Ser. No. 264,965  
5 Claims. (Cl. 15—159)

This invention relates to oriented foamed filaments, fibers and bristles of isotactic polypropylene. More particularly, this invention relates to oriented isotactic foamed polypropylene bristles having a diameter of from 10 to 500 mils and possessing enhanced roundness, reduced diameter variation, and increased yield of bristles per pound, with no significant loss of stiffness or abrasion resistance.

It is well known that filaments of polypropylene may have their properties materially enhanced by drawing or stretching the filaments to increase the molecular orientation along the fiber axis. The resultant stretch oriented filaments are characterized by increased tensile strength, low elongation, and increased stiffness and resiliency.

In the melt extrusion of polypropylene filaments, it is necessary to solidify the filaments by cooling prior to softening for stretch orientation such as by quenching in a non-solvent liquid. Subsequently, the filaments are heat softened and longitudinally stretched to orient them. In stretch orienting heat softened filaments of polypropylene, the filament is often supported by some solid surface after it has been softened, but before it is stretched. For example, the filament may be passed through a heating zone wherein the filaments are heated to a temperature within their softening range by the action of a hot liquid or a hot gas in the heating zone. In order to expose the polypropylene filaments to the fluid source of heat for a period of time sufficient to raise the temperature thereof to a point within its softening range, the filaments are frequently conducted through a sinuous path within the heating zone by means of supporting rolls. Such rolls may themselves be independently heated so that they will serve as the source of heat for heating the filaments. In such a case, the fluid source of heat in the zone may be dispensed with. When polypropylene filaments are passed directly through a heating zone unsupported by rolls or other surfaces while in the zone, there may be provided a device such as a roll assembly on the outside of the zone for snubbing the filaments after they have been heat softened but before they are stretched or drawn.

When a polypropylene filament having a circular cross section is cooled to solidify it subsequent to extrusion, the filament undergoes severe cross sectional distortion. Thus, when an extruded polypropylene filament having a circular cross section is cooled to solidify it prior to softening it for stretch orientation, the filament does not retain its circular cross sectional shape but acquires instead an elliptical or nearly elliptical cross sectional shape. This phenomenon is known as "out of roundness." The degree of out of roundness (i.e., amount of cross sectional distortion) increases as the rate of cooling of the extruded filament increases.

Moreover, the out of roundness is accentuated when the filament, after being heat softened, is supported by a solid surface prior to and/or during the drawing thereof. The tension applied to the filament during the stretching operation while the heat softened filament is supported on a solid surface is responsible for this source of out of roundness.

The out of roundness, or cross sectional distortion, may be so pronounced that the length of the major axis of the elliptical cross sectional shape of the distorted filament may be two or more times greater than the length of the minor axis thereof. This phenomenon may best be illus-

**2**

trated by reference to the relative dimensions of the cross sectional shape of the filament. The relative dimension of the cross sectional shape of a filament or dimensional ratio, is the ratio of the length of the major axis to the length of the minor axis. Thus, if the cross sectional shape of the filament is substantially circular, both axes are substantially the same length and the relative dimension of the cross section or dimensional ratio is substantially unity. However, when the length of the major axis is twice as great as the length of the minor axis, the relative dimension or dimensional ratio is 2.0.

When a non-foamed polypropylene filament is extruded and rapidly cooled, notable diameter variations, as well as crystalline irregularities in the form of large vacuoles within the filament, are found to occur along the length of the filament. The large low strength vacuoles appear to be a result of rapid thermal and crystallization contraction. Although the thermal and crystallization contraction may be controlled to some extent by the use of controlled slow cooling of the filament after extrusion, filaments possessing the best abrasion resistance are obtained by rapid quenching or cooling. When stretch oriented, the low strength vacuole points yield more than normal to the orientation stress and create extreme diameter variations resulting in points of low tensile strength along the filament. The uniform small cells of the foamed filaments of the present invention absorb the thermal and crystallization contraction along the axis to the point where the large vacuoles no longer exist. The foamed filaments maintain a substantially round, uniform diameter throughout the length of the filament thus substantially increasing the tensile strength.

The foregoing described disadvantages are avoided by the practice of this invention which, briefly, comprises producing a dimensionally stable filament consisting essentially of oriented isotactic foamed polypropylene having an effective blow-up of from 1% to about 15%, and having a cross section which is substantially round. Such a filament is produced by preparing a mixture of isotactic polypropylene and a quantity of foaming agent sufficient to produce from about 1% to 15% blow, introducing the mixture into a heating zone, melt extruding a filament from the mixture, quenching or otherwise solidifying the filament, subsequently softening the filament and longitudinally stretching said filament. Prior to and/or during the stretching of the filament, it may be supported on a solid surface.

The preferred polypropylene which may be used in the practice of this invention is isotactic polypropylene which is a high molecular weight (i.e., above about 45,000) solid polymer exhibiting a crystalline X-ray diffraction pattern. Such a polymer has a density between 0.99 and 0.94 and a melting point above about 320° F. These polymers may be prepared by methods now well known in the art such as the procedures described by G. Natta in the Journal of Polymer Science, Vol. XVI, pp. 143 to 154 (1955) and in U.S. Patents 2,882,263; 2,874,153 and 2,913,442.

The preferred foaming agents which may be used in the practice of this invention are those which will decompose at temperatures approximating the extrusion processing temperature of polypropylene. For instance, foaming agents such as 1,1'-azobisformamide (Kempore R-125), 4,4' oxybis (benzenesulfonyl semicarbazide), trihydrazino-sym-triazine (THT), bis-benzenesulfonyl hydrazide (BBSH) and barium azodicarboxylate (Expandex 177) are typical of those which may be used in the practice of this invention.

The foaming agent should be present in an amount sufficient to produce up to 15% blow in the extruded

filament. Percent (%) blow may be defined by the following formula:

$$\text{Percent blow} = \frac{\text{Specific gravity (resin)} - \text{specific gravity (filament)} \times 100}{\text{Specific gravity (resin)}}$$

It has been found that filaments containing up to about 15% blow will give the desired properties of improved dimensional stability and reduced diameter variation with no significant loss of stiffness or abrasion resistance.

The polypropylene, which is preferably in particulate form, is thoroughly admixed with the blowing agent and the admixture is introduced into a heating zone. In the heating zone, the polypropylene is heated to a suitable extrusion temperature above its melting temperature. After the admixture has been heated to said temperature, it may be maintained in gastight environs until it has been extruded to prevent premature blowing. The melt of polypropylene is then extruded into a filament. After the filament has been extruded, it may be solidified as by quenching in a non-solvent bath or by air cooling. Subsequently, it is heat softened by some suitable means. This may be accomplished by conducting it through a heating chamber wherein it is supported, preferably, by a plurality of rolls or equivalent supporting members, the peripheral surface of each providing a supporting surface. The filament may be heated while in the heating zone by means of a fluid source of heat, either gas or liquid, or by means of independently heated rolls. Alternatively, the supporting rolls may be eliminated from the heating zone and the filament passed directly through the zone which is heated by some fluid source of heat, or by radiant heat, the filament being unsupported by any member. The softened filament may be snubbed by means of a suitable device such as a conventional snubbing roll assembly after it leaves the heating chamber but prior to the drawing operation. Thus, the heat softened filament may be supported by the surface of the snubbing device after it leaves the heating zone and while in a softened condition.

After the filament has been softened, it is stretched longitudinally to increase the molecular orientation along the fiber axis. Any amount of stretching will increase the molecular orientation. However, maximum benefits are attained by stretching the filaments from about 6 to about 11 or more times of their length.

The drawn filaments of foamed polypropylene have diameters which range from 10 to 500 mils and preferably from 75 to 250 mils.

The cross sectional shape of the drawn filament prepared according to this invention is substantially the same as that of the undrawn filament after it is extruded but before it is solidified and subsequently heat softened prior to the drawing thereof. That is the relative distance between the midpoint of the cross section and the periphery, or the relative dimensions, remain approximately or nearly the same so that, although the size or area of the cross section are considerably less after drawing, the round configuration remains substantially the same.

The filament or bristle produced according to this invention has a structure such that a major part of the foamed portion is located at the center of the bristle and extends lengthwise therethrough. Since the foamed portion is located at approximately the center area of the filament, the thermal and crystallization contraction, which occurs primarily at this center area is apparently absorbed by the foam, resulting in a rounder filament. Substantially none of the foam is in the outer part. Thus the outer portion of the bristle is continuous and non-porous after extrusion. Other polymers, such as polyethylene, must be drawn in order to obtain a continuous surface.

Uniformly shaped filaments produced by the process of this invention are extremely useful in the production of uniform tufts of bristles in a brush. This results in a

more uniform distribution of wear of the bristles. Moreover, such tufts are more easily mounted in brush heads. Flex action in any direction is much more nearly uniform than in oval filaments—i.e., filaments which have gone out of round during processing. Also, the foamed filaments of this invention possess better flaggability than do non-foamed polypropylene filaments.

The aspects of this invention which are capable of illustration, are shown in the accompanying drawings,

FIG. 1 is an end view of a single bristle made according to the present invention.

FIG. 2 is a schematic view of a suitable overall arrangement of apparatus for carrying out the method of this invention.

FIG. 3 is a schematic view of a section of a modification of the apparatus shown in FIG. 2.

FIG. 4 is a schematic view of another apparatus suitable for carrying out this invention in which the filament is softened in a heating chamber which does not contain any supporting surface in the heating chamber itself.

FIG. 5 is a view of a section of a brush in which the bristles of this invention are adapted for use.

FIG. 1 is an end view of a 10% foamed 80 mil bristle under magnification of 100 $\times$ . The bristle 14 has a structure such that the major part A of the foamed portion is located at the center area of the bristle while the outer part B is continuous and non-porous. Approximately 70% of the foamed portion is limited to not more than 30% of the center area.

30 In FIG. 2, a hopper 10 contains pellets 11 of the polypropylene and foaming agent starting material such as crystalline isotactic polypropylene and Kempre R-125. The pellets 11 may be preheated in the hopper 10 if desired. From the hopper 10 the pellets are conveyed by 35 means of a heated extrusion chamber 12 to a heated non-vented extrusion head 13 which contains an extrusion die 13a. In the extrusion chamber 12, the temperature of the mixture is raised to above the melting point of the polypropylene and above the decomposition point of the foaming agent. It is extruded through suitably shaped orifices in the extrusion die 13a into one or more filaments 14. A preferred extrusion temperature for the isotactic polypropylene is about 480° F. when the filaments 14 are extruded at a linear rate of from about 18 40 to about 50 feet per minute from the orifices, the size of which may range from about 10 mils to about 500 mils in diameter.

In making filaments of isotactic foamed polypropylene, it is advantageous to quench the extruded filaments in order to solidify them. Quenching at a temperature below about 60° F. imparts valuable properties to the drawn polypropylene as described in U.S. Patent 3,059,991 to P. C. Munt (the disclosure of which is incorporated herein by reference). This may be accomplished, as shown in FIG. 2, by placing a quench bath 15 between the extrusion head 13 and the heating chamber 22. The extruded filaments 14 are guided into the quench bath 15, containing a liquid non-solvent for isotactic polypropylene, e.g., water, by a guide roll 16. The bath 15 is maintained in a suitable tank 17 at a temperature of 60° F. or below. Temperatures of about 40° F. are preferred. A much lower temperature, such as 10° F., may be used for the quench bath if precautions are taken to keep the non-solvent from freezing. Thus, a salt water brine at temperatures below 32° F. may be used. An immersion time of from about 8 seconds to about 20 seconds of the filaments 14 in the bath 15 is generally sufficient. The filaments 14 are transported around a stationary pin 18 in the quench bath 15 and then over the roll 19 and into the hot air conditioning oven 22. In the oven, the extruded filaments are transported over a number of rolls 20, which may be heated, in a sinuous or zig-zag path, as heated air is circulated from overhead as indicated by the arrows. As the filaments pass through the heating zone,

each succeeding driven roll 20 over which the filaments 14 pass is driven at a slightly increased peripheral speed from that of the proceeding roll so as to prevent the filaments from sagging appreciably. The primary purpose of the series of driven rolls 20 is to provide a heat exchange relationship between the filaments 14 and the heated air in the oven whereby the filaments are uniformly softened by heat. Since isotactic foamed polypropylene has a softening temperature in the range of from about 260° F. to about 305° F., it is preferred to maintain the temperature in the oven at about 300° F.

After leaving the last and uppermost driven roll 20, the filaments are snubbed with a three roll assembly 21, each roll of which is driven at about the same as or a higher peripheral speed than that of the last driven roll 20. A fast snub roll assembly 23 is provided just outside the oven 22 which is driven at a peripheral speed of about 6 to 11 times that of the assembly rolls 21. Thereby, the filaments 14 are stretched from about 6 to 11 times their length. This increases the molecular orientation along the fiber axis. The drawn, oriented filaments 14 are thereafter collected on a reel 24 which is supported on a frame 25.

FIG. 3 illustrates a modification of the apparatus shown in FIG. 2 in which extruded filaments 14 are solidified by air cooling rather than by quenching. The filaments 14 are passed over the rolls 31 to allow them to solidify prior to being transported into the hot air conditioning oven 22.

In FIG. 4, filaments 40 having a substantially round sectional shape prepared by means, previously described, are passed over a snub roll assembly 39 and thence into the heating chamber 41. A fluid heating means, such as

and the amounts of foaming agent (Kempore R-125) indicated in the following table are fed into a screw extruder of the type shown in FIG. 2 having a 2.5 inch screw diameter. The die plate contains 3 extrusions orifices, each having a circular shape. The non-vented jacket is heated to a temperature of about 480° F. and the filaments are extruded at a linear rate of 35 feet per minute from the orifices. The cross sections of each of the extruded filaments are substantially round. The filaments are then passed through a quench bath maintained at a temperature of about 40° F. to solidify them. They are then fed into a heating chamber and are transported over a series of rolls. Hot air is circulated through the heating chamber, thereby heating the filaments to a temperature of about 300° F. before they leave the heating chamber. After leaving the heating chamber, the filaments are stretched to about eight times their original length to give 80 mil diameter filaments. The cross sections of the drawn foamed filaments are substantially of the same shape as the cross sections of the filaments after they are extruded but before they are quenched and taken over the series of rolls in the heating chamber.

The following table lists the percent blow and the specific gravity as well as the measured volumetric abrasion rate expressed in  $(in.^3/min.) \times 10^{-4}$ , the ratio of the major axis to the minor axis ( $D_2/D_1$ ) and the diameter variation for the filaments produced by each example. As can be seen from this table, the non foamed filament (Example 8) is much more out of round and shows much greater diameter variation than the foamed filaments (Examples 1 to 7). Moreover, the abrasion resistance of the foamed filaments compares favorably with the abrasion resistance of the non foamed filament.

Table

| Example | Amount Foaming Agent, Percent By Weight | Percent Blow | $D_2/D_1$ | Volumetric Abrasion, $in.^3/min.$ | Specific Gravity | Standard Deviation of Diameter from Av. | Percent Variation of Diameter From Av. | Extremes of Variation |
|---------|-----------------------------------------|--------------|-----------|-----------------------------------|------------------|-----------------------------------------|----------------------------------------|-----------------------|
| 1       | 0.01                                    | 4.4          | 1.39      | 0.00055                           | 0.86             | 0.0030                                  | 3.75                                   | $\pm 0.015$           |
| 2       | 0.03                                    | 6.7          | 1.33      | 0.00063                           | 0.84             | 0.0020                                  | 2.3                                    | $\pm 0.010$           |
| 3       | 0.05                                    | 7.9          | 1.265     | 0.00075                           | 0.82             | 0.0026                                  | 3                                      | $\pm 0.012$           |
| 4       | 0.06                                    | 9.8          | 1.24      | 0.00070                           | 0.81             | 0.0010                                  | 1.16                                   | $\pm 0.014$           |
| 5       | 0.07                                    | 11           | 1.20      | 0.00058                           | 0.80             | 0.0022                                  | 2.5                                    | $\pm 0.015$           |
| 6       | 0.09                                    | 13.3         | 1.11      | 0.00065                           | 0.78             | 0.0010                                  | 1.16                                   | $\pm 0.010$           |
| 7       | 0.10                                    | 15.5         | 1.15      | 0.00070                           | 0.78             | 0.0012                                  | 1.5                                    | $\pm 0.008$           |
| 8       | 0                                       | 0            | 1.450     | 0.00060                           | 0.90             | 0.0055                                  | 6                                      | $\pm 0.010$           |

superheated steam, is circulated through the heating chamber. The fluid is introduced into the heating chamber through an inlet and removed through an outlet. The temperature of the heating chamber is maintained at a temperature sufficient to soften the filaments. The heat softened filaments are snubbed by the roll assembly 44 immediately after they leave the heating chamber. These rolls are driven at a slightly higher peripheral speed than the rate at which the filaments are passed into the heating chamber so as to keep the filaments from sagging appreciably while in the chamber. After being snubbed by the roll assembly 44 the softened filaments are drawn to several times of their length by a fast roll 45 which is driven at a peripheral speed of about 6 to 11 or more times that of the snub roll assembly 44. The filaments may then be collected on a conventional reel assembly such as described in FIG. 2.

In FIG. 5, a plurality of bristles 14 are grouped together at one end 50 and inserted into retaining means (i.e. a hole) 51 on a rotary street brush base 52.

The following examples illustrate the best mode contemplated for carrying out this invention:

## EXAMPLES 1 TO 8

In these examples, mixtures of isotactic polypropylene having an average molecular weight of about 100,000, a density of 0.90 and a crystalline melting point of 333° F.,

50

A series of bristles varying in diameters of from about 30 mils to about 500 mils, specifically 30 mils, 250 mils and 500 mils, in thickness as measured after drawing are extruded and quenched as described in the above examples using sufficient blowing agent to achieve a 15% blow. The quench bath is maintained at a temperature of about 40° F. The bristles are then fed into a heating chamber where they are heat softened and stretch oriented. On each foamed bristle, the ratio of the major axis to the minor axis before quenching, as in the 80 mil bristle of Example 1, is about unity. After they are quenched, heat softened and stretched, there is little variation in the dimensional ratio of the cross sections and little diameter variation. The abrasion resistance of these bristles is good.

65

I claim:

1. An abrasion resistant filament consisting essentially of oriented isotactic foamed polypropylene; the ratio of the difference between the specific gravity of said foamed filament and the specific gravity of the original polypropylene from which it is formed, to the specific gravity of the original polypropylene from which said filament is formed having a value of up to 0.15; the ratio of the length of the major axis to the length of the minor axis of the cross section of said filament being not greater than about 1.39;

70

75

the diameter of said filament being substantially constant along the length thereof; said filament having a major part of the foamed portion located at the center area and extending lengthwise through said filament.

2. A filament as defined in claim 1 having a diameter of from 10 to 500 mils.

3. A filament as defined in claim 1 having a diameter of from 75 to 250 mils.

4. An abrasion resistant brush bristle consisting essentially of oriented isotactic foamed polypropylene; the ratio of the difference between the specific gravity of said foamed bristle and the specific gravity of the original polypropylene from which it is formed, to the specific gravity of the original polypropylene from which said bristle is formed having a value of up to 0.15; the ratio of the length of the major axis to the length of the minor axis of the cross section of said bristle being no greater than about 1.39;

5

the diameter of said bristle being substantially constant along the length thereof; said bristle having at least approximately 70% of said foamed portion limited to not more than approximately 30% of the center area of said bristle.

5. A brush containing a plurality of bristles as defined in claim 4.

## References Cited in the file of this patent

## UNITED STATES PATENTS

|           |          |       |                |
|-----------|----------|-------|----------------|
| 2,341,823 | Smith    | ----- | Feb. 15, 1944  |
| 2,659,921 | Osborn   | ----- | Nov. 24, 1953  |
| 2,812,530 | Whitesel | ----- | Nov. 12, 1957  |
| 2,888,415 | Jankens  | ----- | May 26, 1959   |
| 2,905,648 | Haas     | ----- | Sept. 22, 1959 |
| 2,907,096 | Halbig   | ----- | Oct. 6, 1959   |
| 2,913,769 | Kastli   | ----- | Nov. 24, 1959  |
| 2,948,048 | Jankens  | ----- | Aug. 9, 1960   |
| 2,950,495 | Stingley | ----- | Aug. 30, 1960  |
| 3,050,070 | Sidelman | ----- | Aug. 21, 1962  |
| 3,059,991 | Munt     | ----- | Oct. 23, 1962  |